

Patented July 24, 1951

2,561,816

# UNITED STATES PATENT OFFICE

2,561,816

## POLISH

Arthur C. Pabst, Douglaston, and Rudolph J. Holzinger, New York, N. Y., assignors to Socony-Vacuum Oil Company, Incorporated, a corporation of New York

No Drawing. Application December 9, 1948,  
Serial No. 64,441

6 Claims. (Cl. 106—10)

1

The present invention relates to wax polishes and, more particularly, to those polishes known as paste and liquid wax polishes including emulsions.

Presently available wax polishes of either the paste or liquid type, including aqueous emulsions, are prepared employing a petroleum fraction known as mineral spirits or Stoddard solvent, with a boiling range corresponding substantially to the following:

50% minimum at 350° F.

90% minimum at 375° F.

That is to say, at least 50 per cent of the petroleum fraction is distilled when the temperature of the vapors reaches 350 degrees Fahrenheit and at least 90 per cent of the petroleum fraction is distilled when the temperature of the distillation reaches 375 degrees Fahrenheit. The solvent must also meet the requirements that the final boiling point is not greater than 410 degrees Fahrenheit and that the flash point as determined in the Tagliabue closed cup is at least 100 degrees Fahrenheit.

When a solvent having a higher flash point is used the polish so produced requires excessive periods of drying before buffing of the polish coated surface can be attempted. The delay so caused is the result of the lower volatility and consequent lower rate of evaporation of the solvent. On the other hand, solvents of materially lower boiling range, while offering certain advantages such as less offensive odor and a finished preparation of increased body, have not been found satisfactory because of the considerably lower flash point which introduces undesirable hazards into the manufacturing processes and into the use of the finished product.

We have discovered that the deficiencies of the presently commercially available wax polishes can be overcome in a simple but efficacious manner. The wax polishes of the present invention have a sufficiently bland odor that a deodorant or maskant or perfume is not essential to disguise the odor of the product. This seems to

2

be a minor consideration but those who supply these products to the consumer know that a product having an odor to which the consumer objects is not readily salable.

The novel product of the present invention has increased body when compared with conventional prior art products of equal wax content. On the other hand, a product of the same consistency or body as that of the conventional commercially procurable polishes can be obtained at a lower concentration of the active, and generally, more expensive ingredients. While the latter is advantageous from a standpoint of economy, the paste polishes of greater consistency permit a more sparing and evenly distributed application with the result that a more uniform and more durable coating of greater area can be obtained. Similar advantages are gained with liquid polishes together with decreased loss of material through absorption by the cloth pad or applicator ordinarily employed in the application of the wax to the surface to be polished.

Aside from the foregoing advantages resulting from the novel combination of the present invention, the manufacture of wax polishes within the scope of the present invention is simplified and improved.

The wax polishes now offered to the trade commonly are produced in accordance with the following procedure. The waxes are dissolved in the solvent by means of heat and agitation at about 150 to about 200 degrees Fahrenheit. The solution is then cooled to the point of incipient crystallization. The mush so obtained is homogenized, for example by grinding in a colloidal mill, in order to prevent the formation of granular crystalline agglomerates and to promote the formation of a gel structure. The formation of a gel structure ensures the production of a stable homogeneous polishing preparation. Since the solution of waxes must be cooled to incipient crystallization, the higher the temperature at which the solution of waxes "sets" the less forced cooling is required and the lower the expense of the cooling step. Furthermore, the reduced

amount of cooling necessary to reach the "setting" temperature shortens the time during which the batch is held in the cooling vessel prior to grinding and filling the containers. This permits greater production with equipment of given capacity or comparable production with equipment of lower capacity. In other words the capital cost per unit of product produced is lowered.

The higher gelling or setting temperature of the wax polishes within the scope of the invention provides additional advantages. During transit the wax polishes are often subjected to temperatures above the "setting" or "gelling" temperature of polishes presently available to the trade. At the time of application atmospheric temperatures in many localities are above the softening temperatures of polishes now offered to the trade. When the application of wax polishes is attempted at temperatures above the softening point of the wax polish, application becomes difficult or impossible. At temperatures above the gelling temperature, the original gel structure of liquid waxes becomes thin and the particles of wax settle-out rapidly creating a non-homogeneous or heterogeneous product. In more severe cases excessive temperatures during storage or transit tend to cause re-solution of the wax both in liquid and paste type polishes. Upon subsequent cooling the redissolved wax crystallizes without impediment thus destroying the effect of the homogenizing treatment to which the polish was subjected during manufacture, thereby producing an unsatisfactory product. The recrystallization after re-solution usually takes place over a relatively long period of time, thereby frequently giving rise to selective crystallization and attendant segregation and stratification of component waxes. Such a stratification detracts both from appearance and usefulness.

We have discovered that the disadvantages briefly discussed hereinbefore and others known to those skilled in the art can be eliminated or at least markedly reduced by employing a novel solvent for the solid ingredients of the wax polishes. This solvent meets the specification with respect to boiling range set forth hereinbefore and has a rate of evaporation comparable to that of conventional solvents for the preparation of wax polishes. Paste waxes produced in accordance with the following description have a higher milling temperature, a higher melting point, a higher pour point and are harder than prior art wax paste polishes.

Liquid wax polishes produced in accordance with the following description are homogeneous after standing for two weeks at temperatures of about 80 to about 85 degrees Fahrenheit. The polishes are of far greater consistency as indicated by the viscosity at 77 degrees Fahrenheit.

It is an object of the present invention to provide a paste type wax polish having a higher milling temperature, a higher melting point and a more pleasant odor than conventional paste type wax polishes now available to the trade. It is another object of the present invention to provide wax polishes that withstand higher temperatures without softening and permitting higher temperatures during application than conventional wax polishes. It is a further object of the present invention to provide liquid type wax polishes stable for longer periods of time at higher temperatures than conventional wax polishes. Other objects and advantages will become apparent from the following description.

As has been pointed out, a solvent suitable

for use in the preparation of wax polishes of both the paste and liquid type must meet certain specifications with respect to boiling range. In addition, the flash point of the solvent must be sufficiently high to reduce the fire hazard and the rate of evaporation must be sufficiently high to permit satisfactory application of the polish. The novel solvent employed in the described pastes satisfies all of these requirements and, in addition, has a higher "setting" temperature than presently used solvents. In order to provide a basis for comparison, the characteristics of solvents typical of those presently employed to a considerable extent and of the novel solvent are given in Table I.

Table I

|                                      | Mineral Spirits | Novel Solvent |
|--------------------------------------|-----------------|---------------|
| Gravity, °API                        | 47.6            | 48.3          |
| Initial Boiling Pt., °F.             | 312             | 308           |
| 10%, °F.                             | 325             | 318           |
| 50%, °F.                             | 341             | 330           |
| 90%, °F.                             | 364             | 350           |
| Final Boiling Pt., °F.               | 389             | 384           |
| Flash Point:                         |                 |               |
| Tag, closed cup, °F.                 | 103             | 105           |
| Aniline Pt., °F.                     | 129.0           | 128.0         |
| Kinematic Viscosity at 100° F., CSKS | 1.04            | 1.39          |
| Paraffinicity Index                  | 62.7            | 160           |

The novel solvent comprises a mixture of hydrocarbons which exhibits what may be termed superparaffinicity. The novel solvent is most readily obtained by fractionation of the alkylate produced by condensing olefins with isoparaffins in the presence of an acid catalyst such as hydrofluoric acid, phosphoric acid, sulfuric acid and the like. The alkylate so obtained is then subjected to fractional distillation and a fraction having the characteristics set forth below recovered. Such a fraction of alkylate consists primarily of isoparaffins having 9 to 11, averaging 10, carbon atoms per molecule. The novel solvent has the following characteristics:

Table II

|                                               |
|-----------------------------------------------|
| Gravity, °A. P. I. 53.0 to 58.0               |
| Initial boiling pt., °F., 290 to 320          |
| 90%, °F., 355 to 375                          |
| Final boiling pt., °F., 385 to 410            |
| Aniline point, °F., 178.5 to 186.0            |
| Flash point, °F.,                             |
| Tag, closed cup, 110 to 136                   |
| Paraffinicity index, 125 minimum              |
| Odor, bland (like U. S. P. white mineral oil) |

The paraffinicity index (P. I.), as is known, is correlated to the thermo-viscosity or viscosity in centistokes and the A. P. I. gravity by the following equations:

$$P. I. = \left( \frac{\text{Saybolt thermo-viscosity} @ 60^{\circ} \text{ F.}}{5} \right) -$$

$$10(46 - \text{A. P. I. gravity})$$

By using the conversion method developed by L. Brown (Thermo-viscosity of Light Distillates, A. S. T. M. Bulletin, December 1940, page 23) the more common value in centistokes can be substituted for thermo-viscosity in the foregoing equation:

$$\text{Saybolt thermo-viscosity} @ 60^{\circ} \text{ F.} = (\text{Centistokes} @ 100^{\circ} \text{ F.} \times 262) - 39$$

which when substituted in the original equation provides the following equation:

P. I. =

$$[(\text{viscosity in centistokes} @ 100^\circ \text{ F.} \times 262) - 39] - 5$$

10 (46 - A. P. I. gravity)

A comparison of the paraffinicity indices of the novel solvents and commercially available solvents usually referred to as paraffinic solvents establishes that the paraffinicity index distinguishes the hydrocarbon solvents employed in the novel wax polishes described herein over conventional, commercially available presently used solvents.

Table III

|                                  | Viscosity,<br>CSKS <sup>1</sup> @<br>100° F. | Gravity<br>°API | P. I. |
|----------------------------------|----------------------------------------------|-----------------|-------|
| Novel Solvent (I)                | 1.39                                         | 55.5            | 180.0 |
| Novel Solvent (II)               | 1.49                                         | 53.8            | 148.3 |
| Solvent "P" from Penn. Crude     | 0.98                                         | 51.5            | 98.0  |
| Solvent "M" from Mid-Cont. Crude | 1.04                                         | 47.6            | 70.4  |

<sup>1</sup> CSKS = centistokes.

To illustrate the superiority of the novel wax polishes over presently used wax polishes the following comparative tabulation is provided. The solvents employed in preparing the wax polishes for comparative study had the physical characteristics set forth in Table IV.

Table IV

|                                              | Presently<br>used<br>Solvent | Novel<br>Solvent |
|----------------------------------------------|------------------------------|------------------|
| Gravity, °A. P. I.                           | 47.6                         | 55.5             |
| Initial Boiling Pt., °F.                     | 312                          | 317              |
| 10%, °F.                                     | 325                          | 348              |
| 50%, °F.                                     | 341                          | 360              |
| 90%, °F.                                     | 364                          | 368              |
| Final Boiling Pt., °F.                       | 389                          | 386              |
| Flash Pt., °F. (Tag, c. c.)                  | 105                          | 117              |
| Aniline Pt., °F.                             | 129.0                        | 182.5            |
| Kinematic Viscosity at 100° F. (centistokes) | 1.04                         | 1.39             |
| Paraffinicity Index                          | 62.7                         | 160.0            |

Table V (paste waxes)

| Polish                                             | A                  |                    | B                  |                    |
|----------------------------------------------------|--------------------|--------------------|--------------------|--------------------|
|                                                    | Weight<br>per cent | Weight<br>per cent | Weight<br>per cent | Weight<br>per cent |
| Carnauba Wax #3, Refined                           | 3.0                | 3.0                |                    |                    |
| Candelilla Wax, Refined                            | 8.0                | 8.0                |                    |                    |
| Paraffin Wax, Refined (145° F., M. P.)             | 12.0               | 12.0               |                    |                    |
| Microcrystalline Wax                               | 3.0                | 3.0                |                    |                    |
| Mineral Spirits                                    | 74.0               |                    |                    |                    |
| Novel Solvent                                      |                    |                    | 74.0               |                    |
|                                                    | 100.0              |                    | 100.0              |                    |
| Milling Temperature, °F.                           | 102                | 112                |                    |                    |
| Saybolt Melting Pt., °F.                           | 102.75             | 118.0              |                    |                    |
| "Modified A. S. T. M. Melting and Pour Point," °F. | 106.3              | 117.6              |                    |                    |
| A. S. T. M. Cone Penetration:                      |                    |                    |                    |                    |
| @ 77° F., 150 gms., 5 sec., 1/0 mm.                | 122                | 97                 |                    |                    |
| @ 115° F., 150 gms., 5 sec., 1/0 mm.               | Liquid             | 325                |                    |                    |
| Odor                                               | (1)                | (2)                |                    |                    |

<sup>1</sup> Strong, that of petroleum solvent.

<sup>2</sup> Mild, pleasant, that of carnauba wax.

(The Saybolt melting point was determined with the Saybolt improved wax melting apparatus in accordance with the method described in "Tag Manual for Inspectors of Petroleum," 25 24th edition, (1937) C. J. Tagliabue Manufacturing Company. The "Modified A. S. T. M. Melting and Pour Point" conforms essentially to the A. S. T. M. standard method of test for melting point of paraffin wax D87-42 with the following changes: The stirrer described in paragraph 30 3(d) of the test was omitted. The test tube was removed from the bath at each degree Fahrenheit temperature drop and slightly tilted. The reading at which no further movement could be 35 observed due to crystallization was recorded.)

A study of the comparative values recorded in Table V makes it manifest that the paste polishes containing the novel hydrocarbon solvent have characteristics correlated with temperatures 10 to 15 degrees Fahrenheit higher than the corresponding characteristics for paste polishes containing presently used solvents.

The pronounced superiority of liquid type wax polishes containing novel hydrocarbon solvent is 40 evident from a study of the comparative data recorded in Table VI.

Table VI

|                                                                   | I                             | II              | III                          |
|-------------------------------------------------------------------|-------------------------------|-----------------|------------------------------|
|                                                                   | Weight per cent               | Weight per cent | Weight per cent              |
| Carnauba #1 Yellow                                                | 5.00                          | 5.00            | 3.63                         |
| Paraffin Wax (M. P. 130° F.)                                      | 4.00                          | 4.00            | 2.91                         |
| Microcrystalline Wax                                              | 2.00                          | 2.00            | 1.46                         |
| Mineral Spirits                                                   | 89.00                         |                 |                              |
| Novel Solvents                                                    |                               | 89.00           | 92.00                        |
|                                                                   | 100.00                        | 100.00          | 100.00                       |
| Milling Temp., °F.                                                | 86                            | 105             | 103                          |
| Consistency                                                       | Semi-Fluid                    | Gel             | Semi-Fluid                   |
| Appearance after storage for 2 weeks at 80° F.                    | Some solvent separation.      | Homogeneous     | Trace of solvent separation. |
| Viscosity (Brookfield Synchro-electric viscometer), Cps. @ 70° F. | 750                           | Gel             | 750                          |
| Odor                                                              | Pronounced petroleum solvent. | Bland           | Bland                        |
|                                                                   |                               |                 | Total Wax Content, 8.00      |

Again the superiority of the novel wax polishes 70 is to be noted. The desirable bland odor alone of polishes II and III makes these polishes a readily merchantable article. However, it is to be noted that this desirable feature is accompanied by comparable consistency at room temperature for a lower concentration of total solids

Batches of paste type and liquid type wax polishes were made using identical formulations, raw materials and compounding procedures with the exception that in series A the presently used commercially available solvent was used whereas in the series B the novel hydrocarbon solvents were used.

than for polishes employing conventional, presently used solvents. When polishes are prepared with equivalent concentration of total solids, the novel product retains its superiority at higher temperatures than 77 degrees Fahrenheit. Those skilled in the art will also observe that the novel polishes are homogeneous even after storage for two weeks at 80 degrees Fahrenheit whereas the conventional polishes had begun to stratify and segregate.

Those skilled in the art will appreciate that the formulations used for the purposes of the comparative tests are merely illustrative and not limiting and that various changes can be made without departing from the spirit of the invention. Thus, the film forming ingredients of the paste type polish are composed of a hard wax and a soft wax. A hard wax is used to contribute such properties as high luster and good wearing qualities while the soft component contributes other characteristics as, for instance, flexibility and ease of buffing. An additive may or may not be employed in order to accomplish similar purposes or specific objects such as to overcome excessive slipperiness, susceptibility to temperature changes, and so on.

A hard wax in the sense employed herein may be a hard wax, or wax-like substance or a combination or blend of such materials, either of natural origin or else a synthetic or chemically modified product. A hard wax of natural origin may fall in the class of vegetable waxes, as for instance carnauba, candelilla or ouricury wax, or in the class of mineral waxes, such as ozokerite, montan wax or refined or oxidized tank bottom wax. A synthetic or chemically modified material may be one of a number of types widely divergent as to chemical structure. For illustrative purposes, several types might be mentioned; esters, such as fatty acid esters of pentaerythritol, glycol ester of montanic acid (such as ethylene glycol ester of oxidized montanic acid), or hydroxy esters (hydrogenated castor oil), amides such as stearyl amide, polyhydroxy compounds, such as polyethylene glycol of a molecular weight above 1500, preferably in excess of 3000.

A soft wax in the sense employed herein may be a soft wax or wax-like substance or a combination or blend of such materials either of natural origin or else a synthetic or chemically modified product. A soft wax of natural origin may fall in the class of vegetable waxes as for instance Japan wax, in the class of animal waxes such as beeswax or spermaceti, or in the class of mineral waxes, such as paraffin or microcrystalline wax. A soft synthetic or chemically modified material may be or may not be a material similar in chemical composition to the ones described above under hard waxes, except for the difference in physical characteristics, especially hardness. Thus, it may be an ester, hydrocarbon, nitrile, ether or other compound of waxy character.

An additive in the sense employed herein may be substance or a combination or blend of substances that may be obtained from nature, by modification of a natural product or by chemical synthesis. For instance, we might employ a natural resin such as rosin, a chemically modified natural product such as cellulose ethyl ether, or a synthetic resin such as polymethylmethacrylate. Other materials may be soaps, comprising salts of fatty acids with alkalies, alkaline earths or heavy metals, e. g. calcium stearate. Other additives of suitable characteristics may be employed to modify the wax blend or polish-

ing preparation. Accordingly, the novel paste type waxes comprise about 15 to about 35 parts by weight of waxes and about 85 to about 65 parts by weight of a solvent therefor having an initial boiling point of about 290 to about 310 degrees Fahrenheit, a 90 per cent point of about 360 degrees Fahrenheit and a final boiling point of about 390 to about 410 degrees Fahrenheit; a flash point (T. C. C.) of about 100 to about 136 degrees Fahrenheit; and a paraffinic index of at least 125. The novel paste type wax polishes have a melting point of at least about 95 degrees Fahrenheit and the mild pleasant odor of the predominating wax odor. The novel liquid type wax polishes have the consistency of a gel or are semi-fluid, the viscosity of the semi-fluid embodiments of the present invention being about 125 to about 2500. The liquid type wax polishes are distinguished by the homogeneity of the polish after storage at temperatures of about 75 to about 85 degrees Fahrenheit. The composition of both types of novel wax polishes will fall within the following ranges:

| 25 | Polish Type                                                        | Paste, Parts by weight | Liquid, Parts by weight |
|----|--------------------------------------------------------------------|------------------------|-------------------------|
|    | Hard Wax                                                           | about 5 to about 20    | about 2 to about 10     |
|    | Soft Wax                                                           | about 5 to about 25    | about 2 to about 12     |
| 30 | Additive                                                           | about 0 to about 10    | about 0 to about 5      |
|    | Novel solvent                                                      | about 65 to about 85   | about 80 to about 95    |
|    | Milling temperature, °F.                                           | about 95 to about 145  | about 90 to about 130   |
|    | Saybolt melting pt., °F.                                           | about 95 to about 145  |                         |
| 35 | Modified ASTM melting and pour pt., °F.                            | about 95 to about 145  |                         |
|    | Viscosity (Brookfield synchro-electric viscosimeter) cps. @ 77° F. |                        | about 125 to about 2500 |

This application is a continuation-in-part of our application for U. S. Letters Patent Serial No. 713,112, filed November 29, 1946, and now abandoned.

We claim:

1. A paste polish comprising about 15 to about 35 parts by weight of waxes and about 85 to about 65 parts by weight of a hydrocarbon solvent therefor, said solvent consisting essentially of a fraction of alkylate produced by condensing olefins with isoparaffins in the presence of an acid catalyst, said fraction having an initial boiling point of about 290° to about 320° F., a 90% point of about 355° to about 375° F., an aniline point of about 178.5° to about 186° F., a flash point (T. C. C.) of about 110° to about 136° F., a paraffinic index of at least 125 and the bland odor of U. S. P. white mineral oil.
2. A paste polish comprising about 3 weight per cent carnauba wax No. 3, about 8 weight per cent candelilla wax, about 12 weight per cent paraffin wax having a melting point of about 145° F., about 3 weight per cent of microcrystalline wax and the balance to make 100 weight per cent of a hydrocarbon solvent therefor, said solvent consisting essentially of a fraction of the alkylate produced by condensing olefins with isoparaffins, said fraction having an initial boiling point of about 290° to about 320° F., a 90% point of about 355° to about 375° F., a final boiling point of about 385° to about 410° F., an aniline point of about 173.5° to about 186° F., a flash point (T. C. C.) of about 110° to about 136° F., a paraffinic index of at least 125° F., and a bland odor such as U. S. P. white mineral oil; said fraction consisting primarily of isoparaffins having 9 to 11, average 10, carbon atoms per molecule,

3. A liquid polish comprising about 3.6 to about 5 weight per cent carnauba No. 1 wax, about 2.9 to about 4 weight per cent paraffin wax having a melting point of about 130° F., about 1.5 to about 2 weight per cent microcrystalline wax and the balance sufficient to make 100 weight per cent of a hydrocarbon solvent therefor, said solvent consisting essentially of a fraction of alkylate produced by condensing olefins with isoparaffins, said fraction having an initial boiling point of about 290° to about 320° F., a 90% point of about 355° to about 375° F., a final boiling point of about 385° to about 410° F., an aniline point of about 178.5 to about 186° F., a flash point (T. C. C.) of about 110° to about 136° F., a paraffinicity index of at least 125° F., and a bland odor such as U. S. P. white mineral oil; said fraction consisting primarily of isoparaffins having 9 to 11, average 10, carbon atoms per molecule.

4. A liquid polish comprising about 8 to about 11 weight per cent of a mixture of carnauba wax, paraffin wax and microcrystalline wax, and the balance to make 100 weight per cent of a hydrocarbon solvent therefor, said solvent consisting essentially of a fraction of alkylate produced by condensing olefins with isoparaffins, said fraction having an initial boiling point of about 290° to about 320° F., a 90% point of about 355° to about 375° F., a final boiling point of about 385° to about 410° F., an aniline point of about 178.5 to about 186° F., a flash point (T. C. C.) of about 110° to about 136° F., a paraffinicity index of at least 125° F., and a bland odor such as U. S. P. white mineral oil; said fraction consisting primarily of isoparaffins having 9 to 11, average 10, carbon atoms per molecule.

5. A paste polish comprising about 26 weight per cent of a mixture of carnauba wax, candelilla wax, paraffin wax and microcrystalline wax and the balance to make 100 weight per cent of a hydrocarbon solvent therefor, said solvent consisting essentially of a fraction of alkylate produced by condensing olefins with isoparaffins, said

fraction having an initial boiling point of about 290° to about 320° F., a 90% point of about 355° to about 375° F., a final boiling point of about 385° to about 410° F., an aniline point of about 178.5 to about 186° F., a flash point (T. C. C.) of about 110° to about 136° F., a paraffinicity index of at least 125° F., and a bland odor such as U. S. P. white mineral oil; said fraction consisting primarily of isoparaffins having 9 to 11, average 10, carbon atoms per molecule.

6. A wax polish comprising about 2 to about 20 parts by weight of hard wax, about 2 to about 25 parts by weight of soft wax, up to about 10 parts by weight of an additive and the balance sufficient to make 100 parts by weight of a hydrocarbon solvent therefor, said solvent consisting essentially of a fraction of alkylate produced by condensing olefins with isoparaffins, said fraction having an initial boiling point of about 290° to about 320° F., a 90% point of about 355° to about 375° F., a final boiling point of about 385° to about 410° F., an aniline point of about 178.5° to about 186° F., a flash point (T. C. C.) of about 110° to about 136° F., a paraffinicity index of at least 125° F., and a bland odor such as U. S. P. white mineral oil; said fraction consisting primarily of isoparaffins having 9 to 11, average 10, carbon atoms per molecule.

ARTHUR C. PABST.  
RUDOLPH J. HOLZINGER.

#### REFERENCES CITED

The following references are of record in the file of this patent:

#### UNITED STATES PATENTS

| Number       | Name             | Date           |
|--------------|------------------|----------------|
| 2,010,297    | Flaxman          | Aug. 6, 1935   |
| 2,153,161    | Shapiro          | Apr. 4, 1939   |
| 40 2,214,263 | Weihe            | Sept. 10, 1940 |
| 2,311,338    | Holtzclaw et al. | Feb. 16 1943   |
| 2,439,021    | Quigg            | Apr. 6, 1948   |